

No. 624,956.

Patented May 16, 1899.

T. MIDGLEY.

METALLIC TUBING.

(Application filed Nov. 4, 1898.)

(No Model.)



WITNESSES:

Frank L. Ormond.  
W. Parker Reinbold.

INVENTOR

Thomas Midgley,  
BY  
D. L. Reinbold.

ATTORNEY.

# UNITED STATES PATENT OFFICE.

THOMAS MIDGLEY, OF COLUMBUS, OHIO, ASSIGNOR OF TWO-THIRDS TO  
GEORGE C. URLIN AND LEWIS FINK, OF SAME PLACE.

## METALLIC TUBING.

SPECIFICATION forming part of Letters Patent No. 624,956, dated May 16, 1899.

Application filed November 4, 1898. Serial No. 695,476. (No model.)

*To all whom it may concern:*

Be it known that I, THOMAS MIDGLEY, a citizen of the United States, residing at Columbus, in the county of Franklin and State of Ohio, have invented certain new and useful Improvements in Metallic Tubing; and I do hereby declare the following to be a full, clear, and exact description of the invention, such as will enable others skilled in the art to which it appertains to make and use the same.

My invention relates to tubing, has especial reference to that class of tubing which is made of sheet metal, and consists in certain improvements in construction whereby tubing is made of multiple concentric sections of metal metallically joined together and producing seamless tubing, as will be fully disclosed in the following specification and claims.

In the accompanying drawings, which form part of this specification, Figure 1 represents a perspective of two split tubes in position to be assembled; Fig. 2, a transverse section of the tubes assembled; Fig. 3, a like view of the completed tube; Fig. 4, a side elevation of a modified form of the assembled tubing with parts broken away; and Fig. 5 a transverse section of the tubing on line  $x-x$ , Fig. 4.

Reference being had to the drawings and the letters thereon, A indicates the tubing, made of sheet metal, in multiple concentric open or split sections  $a$   $b$ , which are formed of sheets of metal, such as steel or iron, preferably steel, bent into tubular form, with the edges  $c$   $d$  abutting, and are assembled, or one pushed into the other, with the edges of one tube overlapping or out of line with the edges of the other tube, and preferably opposite each other, as shown in Figs. 1 and 2. This disposition of the joints  $e$  of the tubes imparts strength and rigidity to the tubing and reduces the possibility of leaking to a minimum.

The sections  $a$   $b$  are made to fit closely one within the other and may be of different gage sheet metal, according to the weight and strength of tubing required.

To produce a still heavier grade of tubing, the inner section  $a$  is surrounded by a spirally-wound section  $b'$ , and the outer section  $b$  in-

closes the two inner sections, as shown in Figs. 3 and 4. After the multiple sections have been assembled the tubing is immersed in a bath of molten metal, composed of copper and zinc or any suitable brazing or soldering alloy, 55 and allowed to remain in the bath until it has become properly heated and the liquid metal has thoroughly permeated and filled the joints in the tubing and the sections have been permanently joined together by the molten metal 60 and the tubing coated with a non-corroding metal, preferably brass, on its interior and exterior surfaces  $g$  and  $f$ . Tubing thus constructed to all intents and purposes forms brass tubing, the body of which is steel or 65 iron, and produces an article of manufacture which can be substituted for brass tubing at a great reduction in cost and capable of resisting greater strain and rough usage.

The tubing may be used for conducting 70 fluids for various purposes and is adapted for the general use of tubing, such as condenser and boiler tubes and bicycle-frames.

The ends of the tubing may be screw-threaded or flanged for joining or connecting one 75 piece to another in the usual manner.

When used for bicycle-frames, the tubing is made slightly thicker than required when finished, and after it has been metallically joined together in the bath of molten metal 80 the outer coating  $g$  of metal from the bath is removed by the use of acid or by abrasion and the tube drawn through a die and over a mandrel in the usual manner of finishing 85 seamless tubing.

Having thus fully described my invention, what I claim is—

1. Tubing composed of multiple concentric metallic sections, metallically joined together and the inner surface coated with soft metal. 90

2. Tubing composed of multiple concentric metallic sections of hard metal joined together by an interposed body of soft metal and having the inner surface of the tubing coated with soft metal. 95

3. Tubing composed of multiple concentric metallic sections brazed together and the inner surface coated with brass.

4. Tubing composed of multiple concentric metallic sections of hard metal with their 100

joints overlapping, metallically joined together and the inner surface coated with soft metal.

5. Tubing composed of multiple concentric tubular metallic sections one of which is spiral and brazed together.

6. Tubing composed of inner and outer tubular metallic sections and an intermediate spiral tubular section brazed together.

7. Tubing composed of multiple concentric

tubular metallic sections, one of which is spiral, brazed together and the inner surface coated with soft metal.

In testimony whereof I affix my signature in presence of two witnesses.

THOMAS MIDGLEY.

Witnesses:

JOHN W. WILSON,  
E. DE FOREST.